

Patented Oct. 16, 1928.

1,687,799

# UNITED STATES PATENT OFFICE.

PORTER W. SHIMER AND EDWARD B. SHIMER, OF EASTON, PENNSYLVANIA.

## CASTING FERROUS METALS.

No Drawing.

Application filed August 7, 1925. Serial No. 48874.

This invention relates to the casting of ferrous metals, and particularly to a method of treating chaplets used in the making of iron or steel castings whereby a leak-proof union is made between the chaplet and the cast metal.

In making metal castings in molds having cores, studs, anchors or so-called "chaplets" are employed to support the cores and hold them in position during the casting operation, which chaplets are of necessity incorporated within and should form an integral part of the finished casting. In iron founding chaplets of cast iron have been used but these are often melted by the molten iron and the cores displaced as a result. It is therefore common practice to employ chaplets of wrought iron or steel, particularly the latter. Such chaplets, however, without further treatment, unite with difficulty with the molten metal, due to the formation of a surface film of oxide, and the result is that although the chaplets are embedded in the finished casting, they are not integrally united with it and the casting is therefore not leak-proof. In an attempt to overcome this difficulty it is the present practice to coat the chaplets with tin, and the use of copper and silver for this purpose has also been proposed. Although chaplets thus treated are better than untreated ones, the use of such coatings has not solved the problem and imperfect castings very frequently result when chaplets coated with these metals are used. Tin, copper and silver are not metals that have been found to have any useful effect when added to cast iron or steel. Silver in addition is too expensive for general commercial use, and tin, the metal most commonly used to coat chaplets, frequently causes the formation of a spongy zone around the chaplet, and castings in the making of which tin-coated chaplets have been used, often fail to be leak-proof.

In accordance with the present invention we have provided a novel coating for chaplets which is relatively free from the objections noted above. Chaplets so coated become integrally united with the iron or steel cast about them and the resultant castings are substantially leak-proof. In attaining this result we coat the chaplets with metals or alloys which are commonly found in iron and steel and which readily alloy with iron and steel at the casting temperature, particularly the brittle ferro-alloys such as are used

in steel manufacture. The alloys we use melt below the temperature of the molten metal being cast and alloy easily and naturally with the chaplet and the cast metal, thus completely protecting the chaplet from oxidation and causing it to be united with the metal surrounding it to form an integral union and a sound casting.

As an example of one method of carrying out our invention the following is given: Equal parts by weight of spiegeleisen and ferro-phosphorus (for example, spiegeleisen of 20% manganese and ferro-phosphorus of 17%-19% phosphorus) are fused together, cooled and crushed to pass a twenty mesh sieve. The chaplet to be coated is first immersed preferably in a solution of boric acid, in wood alcohol, or other cheap equivalent and then rolled in a mixture of 100 parts of the alloy powder with 75 parts of finely powdered boric acid or its equivalent. The function of the boric acid is to dissolve and flux out rust and metallic oxides, under heat, and thus furnish a clean metallic surface for the alloy to fuse against. Instead of using an alcohol solution of boric acid for wetting the chaplets we have also used successfully water, oil, kerosene, etc. The chaplet, or chaplets, are then heated quickly, in any suitable furnace with a minimum of oxidation (the atmosphere of the furnace should preferably be neutral or slightly reducing) to the temperature of fusion of the alloy, and then quenched in water. The chaplet now has a coating which is alloyed with and is an integral part of it. The chaplet is ready for use. The elements of the coating, namely iron, manganese, phosphorus, carbon silicon and sulphur are those present in all iron and steel, but exist in the coating in proportions which make it fusible at a temperature below that of dull iron, producing a natural union of the coated chaplet with the iron of the casting in which it is embedded. Moreover, manganese and phosphorus are well known and extensively used deoxidizing elements, and thus prevent the formation of the often extremely thin film of oxide between the chaplet and the surrounding metal, which oxidized parting is the main cause of chaplet trouble. As a result of these things a far higher percentage of sound castings is made when using our chaplets than when using the chaplets now commonly employed.

Instead of using an ordinary furnace, for

special work, we may cause the powdered alloy to adhere to the chaplets by use of oil or some equivalent vehicle and then heat them to the temperature required in a case-hardening furnace, the chaplets being packed in boxes surrounded by carburizing compound as in ordinary case-hardening.

In certain cases it might be advantageous to use an alloy having a still lower melting point and for this purpose phosphor-manganese, phosphor-copper, ferro-sulphur, tin, arsenic and other metals or alloys may be added.

When our chaplets are stored for a long time before using, or where they are subjected to conditions favoring rusting, we protect their surfaces in almost any of the methods commonly used.

We claim:

- 20 1. A chaplet for use in ferrous metal founding, having a coating of a ferro-alloy which melts at or below the casting temperature.
2. A chaplet for use in ferrous metal founding, having a coating of an alloy containing iron and manganese which melts at or below the casting temperature.
3. A chaplet for use in ferrous metal founding, having a coating of an alloy containing iron, manganese and phosphorus

which melts at or below the casting temperature.

4. A chaplet for use in ferrous metal founding, having a coating of an alloy made by melting a mixture of spiegeleisen and ferro-phosphorus in substantially equal parts.

5. The method of preparing a chaplet for use, which comprises applying to the chaplet a ferro-alloy in pulverulent form, and a flux, and heating to melt the alloy to form a coating on the chaplet.

6. The method of preparing a steel chaplet for use, which comprises wetting the chaplet, applying a pulverulent mixture of ferro-phosphorus spiegeleisen and a flux, and heating to melt the mixture and form a ferro-alloy coating on the chaplet.

7. A chaplet for use in ferrous metal founding, having a coating of an alloy containing a deoxidizing element which alloy melts at or below the casting temperature.

8. A chaplet for use in ferrous metal founding, having a coating of an alloy containing iron and a deoxidizing element which melts at or below the casting temperature.

In testimony whereof we hereunto affix our signatures.

PORTER W. SHIMER.  
EDWARD B. SHIMER.